

## UNITED STATES PATENT OFFICE

1,999,059

MANUFACTURE OF MERCERIZED CEL-  
LULOSE PRODUCTS

George A. Richter, Berlin, N. H., assignor to  
Brown Company, Berlin, N. H., a corporation  
of Maine

No Drawing. Application May 2, 1931,  
Serial No. 534,708

10 Claims. (Cl. 260—10)

This invention relates to the manufacture of mercerized cellulose products into which cellulose fiber of the character of chemical wood pulp enters as a raw material.

The mercerization of cellulose has long been known and has been applied not only to cotton goods, fabrics, or textile yarns, but also to sheets of interfelted fibers fabricated on machinery of the papermaking type. While it is practicable to mercerize sheets of interfelted fibers (and this has been done in viscose manufacture), nevertheless it is still more practicable and economical to mercerize bulk fiber, such as chemical wood pulp, as large quantities of stock can be handled in apparatus of the simplest kind. Again, the mercerized bulk fiber can be easily washed in countercurrent washing machines, such as used in the pulp industry, which effect a separation of the mercerizing liquor for re-use, without great dilution from the mercerized fiber. Indeed, in a mill producing chemical wood pulps, the standard equipment existing therein, including tanks, pumps, pipes, washers, etc., is serviceable for mercerizing vast quantities of such pulps by treating them as they flow in aqueous suspension through the pulp mill. They may be mercerized and washed at any suitable stage in the pulp mill, for instance before or after bleaching; or the mercerizing treatment may be combined with a bleaching operation.

In accordance with the present invention, cellulose fiber in bulk condition, and more particularly chemical wood pulp, is mercerized and then washed in such condition, whereupon the mercerized and washed pulp is formed into sheets of interfelted fiber on machinery of the papermaking type. By fabricating the sheets from bulk, mercerized fiber, not only am I able to benefit by the economic advantages accruing from mercerizing the bulk fiber, but the resulting sheets are possessed of high porosity and absorbency and are remarkably soft. These characteristics are present in the resulting sheets by virtue of the quality of the mercerized fiber itself; and can be supplemented by forming the sheets and drying them without the use of press-rolls or other devices relied upon in conventional papermaking practice to condense the nascent, wet webs of interfelted fiber. The webs may, in fact, be formed and dried directly on a foraminous carrier or wire,—precaution being taken to avoid stretching or other stress of the webs such as would tend to rupture them. The sheet product of the present invention, although of low tensile strength, is eminently adapted for use as a base or foundation for impregnation with latex, rubber solution, or the like, in the production of artificial leathers. It may also serve as a carrier sheet for other impregnating or bonding media of a wide variety, whose primary function, like that of latex or rubber solution, is to impart such qualities as strength, toughness, and water resistance to the sheet after impregnation and drying. A most important use for the product of the present invention is in the field of cellulose derivative production, such as the xanthate, nitrate, and acetate. Its sheet form means that it can be stored, packed, and shipped economically. The low solution viscosity of the fibers and their mercerized state make for smooth esterification; and the high alpha cellulose content of the mercerized fibers leads to derivatives of the highest quality. In this connection, it is to be observed that the mercerization of the pulp may be readily conducted under conditions to produce a mercerized product which, after washing, has an alpha cellulose content upwards of about 96% (frequently 98%) and a solution viscosity of less than 0.6, but in some instances, however, the mercerizing steps may be performed without drastically lowering the solution viscosity of the fiber, as when the product is to serve as a carrier sheet for impregnating media. For instance, by using a mercerizing liquor for a sufficient period of time at room temperature, chemical wood pulp, such as sulphite, may be converted into the desired product. The use of mercerizing liquors at low temperatures, say, distinctly below freezing, facilitates the attainment of the desired product; and the addition of oxidizing agents, such as hypochlorites or permanganates, to the bleaching liquor promotes the reduction of the solution viscosity of the fiber to the desired low value, i. e., to a solution viscosity less than 0.6. Such a product can be directly and completely xanthated by treatment with the appropriate amount of caustic soda and carbon bisulphide to produce the xanthate, which means that the usual long period of aging the so-called soda cellulose has been dispensed with. When unbleached chemical wood pulp, such as sulphite, is used as the starting material and the mercerized product is intended for making derivatives, such pulp is bleached before or after the step of mercerization. Or sufficient bleach, such as hypochlorite, is added to the mercerizing liquor to exert the desired decolorizing action, in which case the bleach, as already indicated, is distinctly favorable to a reduction in the solution viscosity of the fiber to the low value desired.

In order to attain sheets of uniform formation or texture from the bulk, mercerized fiber on machinery of the papermaking type, one must bear in mind the tendency of mercerized fiber to 5 clot or bunch, and thus to give rise to sheets of markedly irregular density and thickness. In other words, one must guard against the propensity of mercerized fiber to deposit as "wild" sheets on papermaking machines. In order to 10 overcome this difficulty, the mercerized fiber should be beaten and/or jordaned or otherwise mechanically treated, so as to individualize or disassociate the fiber units and thereby to produce a homogeneous suspension, even though in 15 so doing the fibers are drastically cut or shortened and the resulting sheet is made even more tender than it would otherwise be, owing to the inherent, non-hydratable character of the mercerized fiber. The beating action to which the 20 fiber is subjected may to advantage be supplemented by the action of a Jordan or refining engine, whereupon the fiber may be run off on a papermaking machine into sheets of the desired basis weight and compactness. Thus, the sheets 25 may be as light as 25 pounds or as heavy as 200 pounds basis weight. Their compactness may range from 30 to 70, although calendering treatment may increase the compactness to about 100. The basis weight is the weight of 480 sheets, 30 24 x 36 inches. Compactness is determined by dividing the basis weight by the product of the thickness in inches times 100. For instance, a sheet having a basis weight of 40 pounds and a thickness of 0.004 inch possesses a compactness 35 of 100. Such sheets lack those qualities, including strength, tear resistance, folding endurance, etc., demanded in papers intended for use as such, but they answer the requirements sought for in the other important spheres for which they 40 are designed. The sheets because of their softness and resiliency lend themselves to embossing and in some cases may first be impregnated with such media as nitrocellulose lacquers, rubber latex or rubber solutions, casein glues, or the like and 45 then embossed. Or the steps of impregnation and embossing may be reversed in order. It may be additionally mentioned that other factors conducive to uniform sheet formation may be availed of in the production of my product, such as the 50 use of a papermaking machine having a Fourdrinier wet end, the delivery of the mercerized pulp to the machine as a highly dilute suspension, and the use of hot water as the suspension vehicle. The use of hot water evidently tends to set 55 incipiently gelatinized cellulose which may be generated on the fiber as a result of mercerization, and thus to inhibit sticking and bunching of fibers.

I am not unmindful of my Patent No. 1,700,596, 60 issued January 29, 1929, wherein I have disclosed the use of a mixture of mercerized and unmercerized cellulose fiber for forming paper sheets. The product of the present invention, however, is made wholly from bulk, mercerized fiber, and 65 hence represents a uniform product which can undergo uniform esterification. For instance, when mercerized to sufficiently low solution viscosity, it may be xanthated directly, without leaving unxanthated fibers or "whiskers," where- 70 as a portion of the fibers, if unmercerized, being of comparatively high solution viscosity, would remain unxanthated, unless ageing were resorted to, as in the usual viscose process. The reduction in fiber length ensuing from beating and/or jordaning prior to sheeting the all-mercerized

pulp furnish is of marked value in the xanthating or other esterifying process, as the smaller cellulose units are reacted upon to completion in a shorter period of time. In the case of chemical wood pulps, such as sulphite pulp, derived from spruce, which have been converted into uniform sheets by my process, the fiber units in the sheets may have an average fiber length of as low as 0.2 to 0.5 mm., or ranging between about 0.2 to 1.0 mm., as against an average fiber length 10 of about 1.5 mm. in the original pulp. This perhaps best shows why xanthation, for example, can be completely effected sooner than in the usual viscose process, wherein sheets of unbeaten pulp serve as raw material. 15

I have herein spoken about the "solution viscosity" of the fiber. The term "solution viscosity" as applied to cellulose fiber is an arbitrary one, indicative of the viscosity of a cellulose derivative solution preparable therefrom. The solution usually and herein employed as a standard is a cuprammonium cellulose solution of prescribed cellulose concentration, the viscosity being determined by measuring the time of efflux 20 of a definite volume of such solution under standard conditions, through an orifice of standard size. The solution viscosity of fiber is herein given in absolute C. G. S. units, and is determined by measuring the viscosity of a solution of 6 grams 25 of fiber in a cuprammonium solution composed 30 of 225 cc. of 28% ammonia water containing 9 grams of cuprous oxide. The C. G. S. unit is employed because it is definite, denoting a viscosity 100 times that of water at 20° C., where- 35 fore a cuprammonium cellulose solution of standard composition identifying a fiber as having a solution viscosity of 10 is 1000 times as viscous as water at 20° C. Glycerine, which is often referred to when dealing with solution viscosity 40 of cellulose fiber, has a value of between 8 and 10 units. 45

Examples of procedure falling within the purview of the present invention may be practiced substantially as follows:

*Example I.*—An unbleached, ordinary sulphite pulp may be treated as follows: The fiber may be first chlorinated with chlorine water containing from 2% to 3% chlorine, based on pulp, at ordinary temperatures. The chlorinated stock, after washing, may then be subjected to the action 50 of an 18% caustic soda solution at 20° C. for from 10 to 60 minutes. If a product of low solution viscosity is desired, I may have present in the caustic soda solution a suitable amount, say 4% to 8% of sodium hypochlorite bleach or other 55 oxidant, based on pulp. The product, at the end of such a treatment, is white and has an alpha-cellulose content of about 97% to 98%. If bleach is present during the alkaline treatment, the solution viscosity of the product will be as 60 low as .5. If the oxidizing agent is omitted, the solution viscosity of the product will be in the vicinity of 2 to 3. The mercerized fiber after washing may be post-bleached, if a high degree of whiteness is desired. This is generally accomplished 65 by treating the washed pulp with about 1% bleach, based on pulp; and, if the alpha cellulose content is to be maintained at as high a level as possible, this bleaching should take place with the presence of free alkali, such as caustic soda. 70 The final bleached product is thoroughly washed and antichlorated. It may then be shortened in fiber length as by means of a sharp-bladed Jordan and converted into sheet form on a cylinder machine or on a paper machine equipped with a 75

Fourdrinier wire as the instrumentality on which the pulp is sheeted. Care should be taken to avoid stretches of unsupported sheet, particularly when it is in wet form.

5 *Example II.*—I may vary the procedure, as outlined in Example I, by using a more dilute caustic at lower temperatures. For instance, I may use a temperature of say, 0° C., with a 5% to 6% caustic solution. In this case also, I may use 10 oxidants, as may seem best.

15 *Example III.*—If a product of low solution viscosity is not particularly desired, I may use a solution of both caustic soda and sodium sulphide for mercerizing the stock. When this is done, it is necessary to use higher concentration of 20 caustic soda and sodium sulphide, as sodium sulphide is less active as a mercerizing agent than is caustic soda. Low temperatures, such as 0° C., are of advantage in this case. It is evident 25 that no oxidants can be used in conjunction with sodium sulphide on account of the fact that sodium sulphide is a reducing agent and would react with the oxidant.

30 *Example IV.*—The procedure may be practiced advantageously in some cases with an unbleached fiber which has not been pretreated with chlorine water and which is not intended to be post-bleached. For instance, kraft pulp may be treated merely with a mercerizing liquor and then converted into sheet form as hereinbefore described.

I claim:

1. A process which comprises mercerizing cellulose pulp in bulk form, suspending the mercerized pulp in hot water to inhibit a bunching of fibers, and depositing the fibers from said suspension as a uniformly textured, interfelted sheet.

2. A process which comprises mercerizing cellulose pulp in bulk form, washing the mercerized 40 pulp, beating the mercerized pulp in water until the fibers are reduced markedly in fiber length and become substantially homogeneously suspended as substantially individualized fiber units in the aqueous medium, forming the beaten, mercerized pulp into an interfelted sheet devoid of ingredients other than said mercerized pulp, and converting such sheet into a cellulose derivative while in sheet form.

3. A process which comprises treating prebleached cellulose pulp with a mercerizing liquor under conditions to raise the alpha cellulose content of such pulp to upwards of about 96%, washing the mercerized pulp, beating the mercerized pulp in water until the fibers are reduced 50 markedly in fiber length and become substantially homogeneously suspended as substantially individualized fiber units in the aqueous medium, forming the beaten, mercerized pulp into an interfelted sheet devoid of ingredients other than said mercerized pulp, and converting such sheet into a cellulose derivative while in sheet form.

4. A process which comprises treating prebleached cellulose pulp with a mercerizing liquor containing an oxidant under conditions to raise 55 the alpha cellulose content of such pulp to up-

wards of about 96% and to lower its solution viscosity to downwards of about 0.6, washing the resulting mercerized pulp, forming the washed, mercerized pulp into a homogeneous suspension of substantially individualized fiber units, and forming an interfelted sheet substantially devoid of ingredients other than said mercerized pulp.

5 5. As an article of manufacture, a uniformly textured, waterleaf paper sheet made from only bulk, drastically cut, substantially uniformly mercerized cellulose fibers previously substantially uniformly suspended in water as substantially individualized fiber units, as the paper-making material, said sheet being capable of undergoing substantially uniform esterification 10 throughout and said fiber having a solution viscosity of less than 0.6.

15 6. As an article of manufacture, a uniformly textured, waterleaf paper sheet made from only bulk, drastically cut, substantially uniformly 20 mercerized cellulose fibers previously substantially uniformly suspended in water as substantially individualized fiber units, as the paper-making material, said sheet being capable of undergoing substantially uniform esterification 25 throughout and said fiber having an alpha cellulose content of upwards of about 96%.

30 7. As an article of manufacture, a uniformly textured, waterleaf paper sheet made from only bulk, drastically cut, substantially uniformly 30 mercerized cellulose fibers previously substantially uniformly suspended in water as substantially individualized fiber units, as the paper-making material, said sheet being capable of undergoing substantially uniform esterification 35 throughout and said fiber having an alpha cellulose content of about 96% and a solution viscosity of less than 0.6.

35 8. The process which comprises substantially uniformly mercerizing cellulose fibers, forming 40 from such mercerized fibers a substantially homogeneous suspension of substantially individualized fiber units substantially all of which have been mercerized, and forming the fibers into a sheet substantially devoid of ingredients other than 45 said fibers.

45 9. The process which comprises substantially uniformly mercerizing cellulose fibers, forming 50 from such mercerized fibers a substantially homogeneous suspension of substantially individualized fiber units substantially all of which have been mercerized, forming the fibers into a sheet substantially devoid of ingredients other than said fibers, and converting such sheet into a cellulose derivative while in sheet form.

55 10. As an article of manufacture a substantially uniformly textured waterleaf paper sheet made from substantially only bulk, drastically cut, substantially uniformly mercerized cellulose fibers previously substantially uniformly suspended in water as substantially individualized fiber units, as the paper-making material, said sheet being capable of undergoing substantially uniform esterification 60 throughout.

65 GEORGE A. RICHTER.